

Jan. 12, 1937.

C. J. BEAVER ET AL

2,067,169

ELECTRIC CABLE

Filed Jan. 27, 1933

Fig. 1.



Fig. 2.



INVENTOR

Charles James Beaver  
Edward Leslie Davy  
BY  
Byrnes, Stebbins, Parmenter & Blonko

their ATTORNEYS

## UNITED STATES PATENT OFFICE

2,067,169

## ELECTRIC CABLE

Charles James Beaver and Edward Leslie Davey,  
Cheshire, England, assignors to W. T. Glover  
and Company Limited, Manchester, England,  
a British company

Application January 27, 1933, Serial No. 653,763  
In Great Britain February 9, 1932

11 Claims. (Cl. 173—264)

It is well known that in high voltage cables of the paper insulated lead covered type, as at present manufactured, the presence of remanent or occluded air or gas is very undesirable because of the risk of it being ionized at high electric stresses and thereby producing local conditions tending to the breakdown of the dielectric.

By the common method of impregnation, in which the cable, previously lapped with paper, is dried and impregnated in vacuo with oil or compound (hereinafter, for convenience, spoken of as compound), it is recognized that it is impossible to eliminate entirely residual air and gas.

Further, this method imposes comparatively low limits on the viscosity of the impregnating compound in order that it may penetrate the wall of dielectric.

The result is that, while the residual air or gas is usually finely divided and uniformly distributed as very small bubbles or in solution in the impregnating compound of the dielectric when the cable is newly made, and the dimensions of the occlusions are such that the gas is not ionizable until much higher stresses than those corresponding to the working voltage have been applied, the said dimensions are liable to become altered by aggregation after the cable has been heated, so that ionization may then occur at lower stresses.

This aggregation is permitted by the mobile character of the impregnating compound, which is necessitated, as mentioned, by the requirements of penetration in the impregnation process.

On the other hand if it is attempted to impregnate more fully, so that residual gas is much reduced, the dilation of the impregnating compound—unrelieved by gaseous compression in the dielectric—distends the lead sheath when the cable is heated under load, so that on cooling, low pressure spaces, containing gas ionizable under working conditions, tend to form in the dielectric.

In order to overcome these drawbacks of lead distension and/or gas aggregation, producing conditions under which the residual gas in an impregnated paper dielectric may become ionizable under working conditions, in accordance with the present invention, spaces of definite and substantially invariable dimensions are provided for the gas which is retained in the cable under such a pressure (substantially above atmospheric pressure) having regard to the dimensions of the spaces that it is not ionizable in the conditions under which the cable will work. The dimen-

sions are assured (1) by forming the spaces in the process of lapping on the paper layers so that they are determined radially by the thickness of the paper, and longitudinally by the spacing of the lappings in each layer, and (2) by providing that these spaces are substantially clear of free compound; that is, the compound is present only in the paper and on its surfaces and is retained there.

In preparing the paper for use in the manufacture of a cable in accordance with the present invention it is impregnated before application to the conductor with a compound having such a setting point as to ensure that physical stability of the impregnated paper is maintained up to a temperature well above the maximum reached in the working conditions of the cable. The impregnation may, for instance, be carried out as set out in the specification of U. S. A. Patent No. 1,752,972 or of U. S. A. Patent No. 1,958,984.

In addition to the impregnation the paper may be provided with a lubricating film as described in the said specifications. This film is preferably applied to one side of the paper only and is of very small thickness. It may, for instance, consist of a coating of petroleum jelly having a high viscosity and set point.

The impregnating treatment of the cable is completed by the operations on the paper above described. There is no subsequent addition of compound, either during the lapping of the paper or to the completed paper dielectric.

An example of a cable embodying the present invention is illustrated diagrammatically in the accompanying drawing of which Figure 1 shows a transverse section and Figure 2 shows a longitudinal section.

In this cable the conductor 1 is covered with a thin metal tape or foil 2 and is lapped with layers or laminae of paper strip indicated by the reference numerals 3, 4 and 5. Over the outside of this dielectric material is placed a metallized layer 6 (preferably perforated) and over this the lead sheath 7 is applied. To the outside of the lead sheath is applied a metal reinforcing tape 8 and this is protected in the usual way by layers of impregnated fabric 9.

The metal tape 2, the metallized paper 6, the reinforcing tape 8 and the fabric layers 9 will as usual be lapped on helically. No attempt has been made to show this in the drawing.

The thin metal tape 2, lapped on the conductor 1, performs the known function of reducing local intensities of electric stress and also gives a def-

5

10

15

20

25

30

35

40

45

50

55

inite inner cylindrical surface to the dielectric layer.

Instead of using this tape the desired results can be obtained by forming (either before or after stranding) the component wires of the outermost layer of the conductor in such a way as to give a smooth outer surface to the conductor. Alternatively a thin lead tube covering the conductor as a whole may be used as described in 10 the specification of U. S. A. Patent No. 1,256,863.

It will be seen from the drawing how the dimensions of the gas spaces 10, between adjacent turns of the paper are fixed by (1) the spacing apart of adjacent turns and (2) by the thickness of 15 the paper laminae. The former determines the longitudinal width of the spaces and the latter, the radial depth thereof. The metal tape 2 forms the inner surface of the innermost gas spaces. The metallized paper layer 6 forms the outer surface 20 of the outermost gas spaces. It will be understood that any gas which may be found in spaces between the metallized paper layer 6 and the sheath 7 will not be subject to electric stress. The same remark applies to the gas between the 25 tape 2 and the wires of the conductor 1 and in the interior of this conductor.

From the preceding description of a single core cable it will be readily recognized how the invention may be embodied in cables having more than 30 one core. It will be understood that the precautions taken to secure the absence of free compound must be extended to the material used for the fillers between the cores (where these are impregnated) as well as to any belt insulation 35 which may be used in addition to the insulation of the individual cores.

Accurate predetermined of the spaces for the gas formed between adjacent turns of each helically applied layer of impregnated paper results from the choice of a suitable thickness of 40 paper and the staggering of successive layers so that none of the helical spaces are directly superposed. This last condition can be attained, for instance, by lapping the layers of impregnated 45 paper on the cable by means of a machine of the type in which the cable rotates and the heads from which the paper is paid out are stationary and the relative positions of the paper strips accurately maintainable and under continuous 50 observation. Such a machine is described in the specification of U. S. A. Patent No. 1,591,736. It is to be understood however that the immersion of the cable in compound during lapping, which is described in that specification, is not to be 55 employed in the present case. The strips or wrappings of the preimpregnated paper are lapped on the cable in air which is preferably kept below normal humidity and the cable is then sheathed with lead or lead alloy with or 60 without reinforcement. After this the air enclosed in the dielectric, which is chiefly located in the spaces provided between the turns of paper, may be evacuated and replaced by an inert dry 65 gas, such as nitrogen, carbon dioxide or other suitable gas. The process or removal of air and filling with gas may be facilitated by a repeated flooding and exhausting of the gas into and from the cable and by the application of heat to the 70 cable intermittently or continuously, either by external means or by the passage of current through the conductor or conductors or by both of these. Finally the gas is forced in under pressure, the cable having been sealed at the ends in order to retain the pressure. When the cable is 75 in service a gas cylinder can be left connected to

the cable through a non-return valve so as to maintain the pressure within the cable if accidental lowering should occur.

The gas pressure is chosen in relation to the thickness of gas films formed in the dielectric, 5 which is determined by the thickness of the individual layers of paper, so that according to well known laws the ionization point of the films of gas exceeds by a predetermined margin the working 10 stress in the dielectric. 10

Instead of replacing the air by some other gas the cable may be finally filled with dry air under pressure, but a preliminary evacuation and heating may also be required in this case.

The choice of the radial dimensions of the gas 15 spaces and of the gas pressure will depend upon a number of conditions. It will however generally be advantageous to make the gas spaces of small radial dimensions, for instance, one or one and a half thousandths of an inch. With such dimensions and with only a comparatively moderate 20 gas pressure, for instance, fifteen pounds per square inch above atmosphere, very material increase in the ionization point can be obtained in cables constructed in accordance with the invention. It is of course possible to use other dimensions and higher pressures, the choice of pressure being materially affected by the cost of 25 strengthening or reinforcing the sheath which it may require. This may, however, in some cases 30 be offset by the reduction in diameter which can be obtained by increase in pressure.

By increasing the thickness of the layers or wrappings of paper from the conductor outwards, 35 the radial dimensions of the gas spaces may also be increased, taking advantage of the fact that the intensity of electric stress decreases from the surface of the conductor outwards. This is indicated diagrammatically in the drawing where three different thicknesses of paper are intended 40 to be indicated for the regions 3, 4 and 5 respectively. Using a gas pressure of about 100 lbs. per square inch suitable values for the thicknesses of the paper laminae or wrappings for this example are:— 45

Region 3 a thickness of 1.75 thousandths of an inch.

Region 4 a thickness of 2.5 thousandths of an inch.

Region 5 a thickness of 3.75 thousandths of an 50 inch.

The type of cable illustrated in the drawing may be used with gas pressures up to 200 lbs per square inch and considerably higher.

In the improved cable it is provided that the 55 solid portion of the dielectric, namely the impregnated paper, is physically stable under most severe working conditions and the gaseous content of the cable is prevented from undergoing 60 appreciable alteration of form, position and dimensions and therefore from becoming ionizable. Further the compressibility provided by the gaseous content of the cable prevents the application 65 of excessive pressure to the reinforced sheath such as would produce permanent distension.

What we claim as our invention and desire to secure by Letters Patent is:—

1. An electric cable comprising a conductor, an enclosing sheath and a dielectric layer between 70 the conductor and the sheath, said layer comprising impregnated paper and a gas at a pressure substantially above that of the atmosphere, which gas occupies spaces of definite and substantially invariable dimensions and sub- 75

stantially clear of free compound under all working conditions, which spaces are distributed through the dielectric layer and which spaces are of increasing radial dimensions from the 5 conductor outwards.

2. An electric cable comprising a conductor, a sheath and a dielectric layer between the conductor and the sheath, the said layer comprising turns of impregnated paper spaced apart to provide intervening compound-free spaces, the thickness of the paper and the corresponding radial 10 dimensions of the spaces increasing from the conductor outwards, and gas under pressure substantially above that of the atmosphere filling 15 said spaces.

3. An electric cable comprising a conductor, an enclosing sheath and a dielectric layer between the conductor and the sheath, said layer comprising wrapped paper impregnated with highly viscous compound, and gas at a pressure substantially above that of the atmosphere, which gas occupies spaces in the dielectric layer of dimensions predetermined in size so as to avoid ionization 20 of gas and which spaces are substantially invariable in position and dimensions and are substantially clear of free compound under all working 25 conditions, which spaces are distributed through the dielectric layer.

4. An electric cable comprising a conductor, an enclosing sheath and a laminated dielectric layer between the conductor and the sheath, said layer comprising wrapped paper impregnated with highly viscous compound, and gas at a pressure substantially above that of the atmosphere, which gas occupies spaces in the dielectric layer 30 of substantially invariable dimensions which are bounded by the turns and laminae of the paper, which spaces are substantially clear of free compound under all working conditions.

40 5. An electric cable comprising a conductor, an enclosing sheath and a laminated dielectric layer between the conductor and the sheath, said layer comprising paper impregnated with a compound which has a high setting temperature above the 45 range of the working temperature of the cable and which compound is thereby retained in and confined to the paper under all working conditions, said layer also comprising gas at a pressure substantially above that of the atmosphere, 50 which gas occupies spaces of substantially invariable dimensions, which spaces are bounded by the turns and laminae of the paper.

6. An electric cable comprising a conductor, an enclosing sheath and a dielectric layer between the 55 conductor and the sheath, said dielectric layer comprising wrapped paper impregnated with a highly viscous compound, said layer having helical spaces therein of mechanically predetermined locations and dimensions such that the dielectric 60 strength of any radial dimension of said layer is predetermined, said spaces having gas therein at a pressure above atmospheric, the spaces being formed between edges of adjacent turns of paper and between surfaces of concentric wrappings.

65 7. An electric cable comprising a conductor, an enclosing sheath and a dielectric layer between

the conductor and the sheath, said layer having helical spaces therein of mechanically predetermined locations and dimensions, said dielectric layer comprising wrapped paper impregnated with a highly viscous compound, the spaces being 5 formed between edges of adjacent turns of paper and between surfaces of concentric wrappings, said spaces having gas therein at a pressure above atmospheric, the dielectric strength of each part of said layer being predetermined by the dimensions of the spaces and the gas pressure. 10

8. An electric cable comprising a conductor, an enclosing sheath and dielectric material between the conductor and the sheath, said material being constituted by definitely spaced turns and layers 15 of paper tape of predetermined thickness, which tape is fully impregnated with a highly viscous compound which is confined to the paper under all working conditions, and gas at a pressure substantially above that of the atmosphere occupying 20 all the spaces between the turns and layers of paper tape.

9. An electric cable comprising a conductor, an enclosing sheath and dielectric material between the conductor and the sheath, said material being constituted by definitely spaced turns and layers of paper tape of predetermined thickness, which tape is fully impregnated with oil compound which has a setting point higher than 25 the working temperature of the cable, whereby 30 the compound is confined to the paper under all working conditions and gas at a pressure substantially above that of the atmosphere occupying all 35 the spaces between the turns and layers of paper tape.

10. An electric cable comprising a conductor, an enclosing sheath and dielectric material between the conductor and the sheath, said material being constituted by turns and layers of paper tape with spaces of definite and substantially invariable dimensions between the turns and of increasing radial dimensions from the conductor outwards, said tape being fully impregnated with compound which is confined to the paper under all working conditions and by a gas 40 at a pressure substantially above that of the atmosphere occupying all the spaces between the turns and layers of paper tape.

11. An electric cable comprising a conductor, an enclosing sheath and dielectric material between the conductor and the sheath, said material being constituted by turns and layers of paper tape with spaces of definite and substantially invariable dimensions between the turns and of increasing radial dimensions from the conductor outwards, said tape being fully impregnated with oil compound which has a setting point above the range of the working temperature of the cable, whereby the compound is confined to the paper under all working conditions 55 and by a gas at a pressure substantially above that of the atmosphere occupying all the spaces between the turns and layers of paper tape.